

## UNITED STATES PATENT OFFICE

JOHN H. MARTIN, OF BALDWIN, NEW YORK

## PREPARATION OF FUR FOR SHRINKING AND FELTING

No Drawing.

Application filed April 16, 1927. Serial No. 184,437.

In the preparation of fur hair or fur (as it may be designated for brevity) for felting and for the shrinkage which must accompany the felting, particularly in the manufacture of hats, the fur, either on the skin or after its removal from the skin, is subjected to the action of chemicals which so affect the character of the fur as to promote the shrinking and the felting, the chemical employed, generally in solution, being sometimes brushed into the fur on the skin, the fur being subsequently removed from the skin, and being sometimes used as a bath in which the fur is immersed after removal from the skin. After treatment with the chemical, the fur is dried and is thereafter subjected to shrinking and felting and dyeing processes, to which the treatment referred to is preliminary. The method here-  
tofore employed and even now commonly employed has involved the use of nitrate of mercury, which gives satisfactory results so far as the shrinking and felting qualities of the fur are concerned, but is known to be exceedingly harmful to those who apply it and to those who handle the fur in subsequent processes. Other chemicals, such as sodium peroxide, have been proposed, but have been found to give less satisfactory results so far as concerns the effect on the fur. Still other chemicals have been proposed and have been found to give satisfactory results, although the discovery of their effectiveness has been so recent that they have not yet come into wide use. In the further investigation of the subject and in the development of the present invention, it has been found that a salt of manganese in solution, either organic or inorganic, will produce results not only fully equal to that produced by nitrate of mercury without its harmful effect, but even superior in the felting quality of the fur and in the absence of undesirable effects on color or otherwise. The solution of the salt of manganese may be either neutral or acid, depending on the characteristics of the fur to be treated, and may be also of different degrees of concentration, depending also on the nature of the fur. As examples of embodiments of the invention, the following are

noted, it being understood that the solution is applied to the fur in the usual manner, either to the fur before it is removed from the skin or to the fur after it is removed from the skin. As a neutral inorganic solution, a four (4) percent solution of nitrate of manganese has been found to give satisfactory results. If the nature of the fur is such as to give better results with an acid solution, two (2) percent of an acid, such as nitric acid, for example, may be added to the four (4) percent solution of nitrate of manganese. As an example of a neutral organic solution, a five (5) percent solution of lactate of manganese may be employed and this may be rendered acid, if conditions require, by the addition of a small percentage, say two or three percent, of some acid, such as lactic acid, for example.

I claim as my invention:

1. The improvement in the art of preparing fur for shrinking and felting, which consists in subjecting the fur to the action of a solution of a salt of manganese which has manganese as its base.

2. The improvement in the art of preparing fur for shrinking and felting, which consists in subjecting the fur to the action of a neutral solution of a salt of manganese which has manganese as its base.

3. The improvement in the art of preparing fur for shrinking and felting, which consists in subjecting the fur to the action of a solution of an organic salt of manganese.

This specification signed this 15th day of April A. D. 1927.

JOHN H. MARTIN.

90

95

100